

Nov. 13, 1951

A. H. DAANE ET AL

2,574,627

URANIUM-COBALT ALLOY

Filed Aug. 26, 1947



INVENTORS:

Adrian H. Daane  
William K. Noyce

By:

Robert A. Lourdes  
Attorney

## UNITED STATES PATENT OFFICE

2,574,627

## URANIUM-COBALT ALLOY

Adrian H. Daane, Ames, Iowa, and William K. Noyce, Fayetteville, Ark., assignors to the United States of America as represented by the United States Atomic Energy Commission

Application August 26, 1947, Serial No. 770,624

1 Claim. (Cl. 75—134)

1

The present invention is concerned with binary uranium-base alloys and more particularly relates to binary uranium-base alloys containing cobalt.

Uranium metal is extremely corrodible, oxidizes readily and may even ignite spontaneously when exposed to air at room temperature.

An object of the present invention is to improve the physical-metallurgical properties of uranium metal so as to enhance the corrosion resistance of uranium and to render the same useful for various purposes for which uranium metal heretofore has not been satisfactory.

Another object of this invention is to produce binary uranium-cobalt alloys which are useful in the construction of neutronic reactors.

A further object of the invention is directed toward the formation of new and novel compositions of binary uranium-cobalt alloys to be used as additives in the formation of more complex alloys containing uranium and cobalt.

Other objects of the present invention will be apparent from the following description taken with the accompanying drawing in which the single figure is a phase equilibrium diagram defining the uranium-cobalt system.

In accordance with the present invention the enhancement of chemical inertness of uranium metal is accomplished by the alloying effects of cobalt which tends toward decreasing corrosive attack by chemical reagents. In addition, by such alloying, uranium compositions are obtained in a form having a much lower melting point than uranium metal.

The present invention is particularly concerned with new and novel compounds of binary uranium-cobalt alloy compositions wherein the cobalt atomic per cent content is less than 50 atomic per cent of the combined uranium-cobalt composition. It was found when preparing low cobalt content alloys of uranium that the uranium liquidus temperature was lowered rather rapidly, as appears in the uranium-cobalt equilibrium diagram of the drawing, by the addition of cobalt until a eutectic composition of 34 atomic per cent cobalt was reached, the eutectic having a melting point of 734° C. The eutectic composition of 34 atomic per cent cobalt with uranium shows a lowering of the melting point of uranium by approximately 400° C.

Referring to the equilibrium diagram, the compound, U<sub>6</sub>Co (14.3 atomic per cent cobalt), which separates as a primary phase in alloys containing less than 34 atomic per cent cobalt is a highly crystalline metal which is formed by a peritectic

reaction at 826° C. In the alloys in which U<sub>6</sub>Co is present, the primary phase of the peritectic reaction appears to go to completion. Thermal and X-ray data indicate that there is no detectable solubility of cobalt in uranium in the primary phase.

The alloy compound U<sub>6</sub>Co is an extremely crystalline phase which can be separated from lower cobalt content alloys of uranium either mechanically or chemically since this compound is not attacked very rapidly by nitric acid. Single crystal diagrams were taken of this phase and the unit cell dimensions of this phase were determined from photomicrographs of isolated needles rotated about the needle (four-fold) axis. It was found that the compound U<sub>6</sub>Co was body centered, tetragonal with the following constants:

$$a_0 = 10.34 \pm 0.02 \text{ \AA}$$

$$c_0 = 5.20 \pm 0.02 \text{ \AA}$$

The density is about 17.7 grams per cubic centimeter, and the volume of a unit cell equal to 550 Å<sup>3</sup> containing 24 uranium atoms and 4 cobalt atoms.

Thermal and microscopic data gave very definite evidence when extending the cobalt atomic per cent content beyond the 34 atomic per cent cobalt eutectic and approaching 50 atomic per cent cobalt that a compound having the formula, UCo, existed. The compound, UCo, 50 atomic per cent cobalt composition decomposed peritectically at 805° C. This compound has a unit cell volume of about 255.4 Å<sup>3</sup> which contains 8 molecules per unit cell to give a density of about 15.4 grams per cubic centimeter.

The alloys of the present invention were prepared from uranium metal having a purity greater than 99.9 per cent and of cobalt metal of 99.9 per cent purity. These metals were melted together in beryllia crucibles in vacuo by means of induction heating. Each alloy mass, weighing about 250–450 grams, was held at about 1500° C. for 20 minutes to allow the melt to come to equilibrium. Thermal data were taken by remelting the alloys and cooling at rates of about 6° to 7° C. per minute in the range of about 1000° C. with correspondingly lower rates at lower temperatures.

50 The alloys were prepared for microscopic examination by mechanical polishing techniques and electrolytic polishing using a phosphoric acid-ethylene glycol-ethyl alcohol solution.

The 34 atomic per cent eutectic alloy of uranium and cobalt affords a low melting uranium

alloy, exhibits high resistance to oxidation, and possesses a high density which makes this alloy a very suitable alloying additive for the preparation of more complex alloys containing uranium. When the 34 atomic per cent cobalt eutectic of uranium is added to a ladle of molten steel, nickel or copper, it rapidly sinks and alloys with the molten bath without excessive oxidation and loss of expensive uranium. Furthermore, the chemical resistance to acid, such as nitric acid, indicates that uranium-cobalt alloys, with or without the addition of other elements, constitute a new series of corrosion-resisting materials which offer unique advantages over uranium. It should be noted that the preferred corrosion-resistant uranium-cobalt binary compositions are contained in a range from about 4 atomic per cent cobalt to about 40 atomic per cent cobalt.

It should be noted that the addition of 5 atomic per cent of cobalt to uranium gives a reduction in the melting point of uranium of approximately 50° C. The decrease of melting point is practically linear to approximately 20 atomic per cent cobalt and then the rate of decrease in the melting point of uranium becomes somewhat less.

All of the alloys above described, in addition to the physical-metallurgical advantages, exhibit resistance to corrosion far superior to that of uranium metal.

It should be noted that the invention is primarily concerned with binary alloy compositions consisting of uranium and cobalt. Since ura-

nium is an essential component in the construction of neutronic reactors, it is extremely important to substantially decrease the corrodibility of uranium metal without introducing a large quantity of neutron absorbers other than the essential alloying agent, cobalt, which has a relatively low neutron absorption cross-section.

It will be understood that the particular alloy composition described above should not be deemed to constitute the limits of the invention. The scope of the invention is defined in the appended claim.

What is claimed is:

A composition of matter consisting of an intermetallic compound of uranium and cobalt defined by the formula:  $U_xCo$  having a density of about 17.7 grams per cubic centimeter.

ADRIAN H. DAANE,  
WILLIAM K. NOYCE.

#### REFERENCES CITED

The following references are of record in the file of this patent:

Friend, "Textbook of Inorganic Chemistry," vol. VII, part III, page 286. Published in 1926 by Charles Griffin & Co., Ltd., London.

Hansen, "Aufbau der Zwerstofflegierungen" 1936. Photo-Lithoprint Reproduction by Edwards Brothers, Inc., Ann Arbor, Mich., 1943, pages 515 and 959.